



US009446504B2

(12) **United States Patent**  
**DiGiovanni**

(10) **Patent No.:** **US 9,446,504 B2**  
(45) **Date of Patent:** **Sep. 20, 2016**

(54) **POLYCRYSTALLINE COMPACTS  
INCLUDING INTERBONDED  
NANOPARTICLES, CUTTING ELEMENTS  
AND EARTH-BORING TOOLS INCLUDING  
SUCH POLYCRYSTALLINE COMPACTS,  
AND RELATED METHODS**

E21B 2010/561; E21B 10/567; C22C 26/00;  
C22C 2026/008; C22C 2026/005; C22C  
2026/007; C22C 2026/003; C22C 2200/04  
See application file for complete search history.

(71) Applicant: **Baker Hughes Incorporated**, Houston, TX (US)

(56) **References Cited**

U.S. PATENT DOCUMENTS

3,745,623 A 7/1973 Wentorf, Jr. et al.  
4,224,380 A 9/1980 Bovenkerk et al.

(Continued)

(72) Inventor: **Anthony A. DiGiovanni**, Houston, TX (US)

FOREIGN PATENT DOCUMENTS

EP 1253123 A1 10/2002  
WO 2004078641 A1 9/2004

(Continued)

(73) Assignee: **Baker Hughes Incorporated**, Houston, TX (US)

OTHER PUBLICATIONS

(\*) Notice: Subject to any disclaimer, the term of this patent is extended or adjusted under 35 U.S.C. 154(b) by 86 days.

Arima, Makoto, et al., "Diamond nucleation and growth by reduction of carbonate melts under high-pressure and high-temperature conditions," *Geology*, vol. 30, No. 8, pp. 691-694, Aug. 2002.

(Continued)

(21) Appl. No.: **14/444,515**

(22) Filed: **Jul. 28, 2014**

(65) **Prior Publication Data**

US 2014/0332287 A1 Nov. 13, 2014

*Primary Examiner* — Cathleen Hutchins

(74) *Attorney, Agent, or Firm* — TraskBritt

**Related U.S. Application Data**

(63) Continuation of application No. 13/226,127, filed on Sep. 6, 2011, now Pat. No. 8,800,693.

**ABSTRACT**

(60) Provisional application No. 61/411,355, filed on Nov. 8, 2010.

Poly-crystalline compacts include non-catalytic, non-carbide-forming particles in interstitial spaces between inter-bonded grains of hard material in a polycrystalline hard material. Cutting elements and earth-boring tools include such polycrystalline compacts. Methods of forming polycrystalline compacts include forming a polycrystalline material including a hard material and a plurality of particles comprising a non-catalytic, non-carbide-forming material. Methods of forming cutting elements include infiltrating interstitial spaces between interbonded grains of hard material in a polycrystalline material with a plurality of non-catalytic, non-carbide-forming particles.

(51) **Int. Cl.**

**E21B 10/46** (2006.01)  
**E21B 10/55** (2006.01)

(Continued)

(52) **U.S. Cl.**

CPC ..... **B24D 3/10** (2013.01); **B24D 99/005**  
(2013.01); **E21B 10/567** (2013.01); **E21B  
10/5735** (2013.01)

**20 Claims, 3 Drawing Sheets**

(58) **Field of Classification Search**

CPC .. E21B 10/46; E21B 2010/545; E21B 10/55;





(56)

## References Cited

## OTHER PUBLICATIONS

- Itoh, M., et al., "Amorphous carbon nitride film preparation by plasma-assisted pulsed laser deposition method," *Appl. Phys. A*, vol. 79, pp. 1575-1578, 2004.
- Kidalov, S.V., et al., "Thermal conductivity of nanocomposites based on diamonds and nanodiamonds," *Diamond & Related Materials*, vol. 16, pp. 2063-2066, 2007.
- Li, Junjie, et al., "Field emission enhancement of amorphous carbon films by nitrogen-implantation," *Carbon*, vol. 42, pp. 2309-2314, 2004.
- Li, Q.Y., et al., "Photocatalytic characterization of silica coated titania nanoparticles with tunable coatings," *Journal of Nanoparticle Research*, vol. 7, pp. 295-299, 2005.
- Liu, Huimin, et al., "Diamond Chemical Vapor Deposition, Nucleation and Early Growth Stages," Dept. of Chemical and Vioresource Engineering, Colorado State University, ISBN 0-8155-1380-1, Noyes Publications, 198 pages, 1995.
- Liu, Huimin, et al., "Nucleation Kinetics of Diamond on Carbide-Forming Substrates during Chemical Vapor Deposition," *J. Electrochem. Soc.*, vol. 143, No. 3, pp. 1104-1109, Mar. 1996.
- Liu, Huimin, et al., "Studies on nucleation process in diamond CVD: an overview of recent developments," *Diamond and Related Materials*, vol. 4, pp. 1173-1188, 1995.
- Majetich, S.A., et al., "Preparation and properties of carbon-coated magnetic nanocrystallites," *Phys. Rev. B*, vol. 48, pp. 16845-16848, 1993.
- Meilunas, R.J., et al., "Diamond Nucleation on Surfaces Using Carbon Clusters," Office of Naval Research, Technical Report No. 12, Dept. of Materials Science and Engineering, Northwestern University, prepared for publication in the *Journal of Materials Research*, 61 pages, May 1993.
- Osipov, A.S., et al., "Rapid sintering of nano-diamond compacts," *Diamond & Related Materials*, 4 pages, 2009.
- Qian, J., et al., "Graphitization of diamond powders of different sizes at high pressure-high temperature," *Carbon*, vol. 42, pp. 2691-2697, 2004.
- Qian, J., et al., "Micron diamond composites with nanocrystalline silicon carbide bonding," *J. Mater. Res.*, vol. 18, No. 5, pp. 1173-1178, May 2003.
- Sadangi, Rajendra K., et al., "WC-Co-Diamond Nano-Composites," *NanoStructured Materials*, vol. 12, pp. 1031-1034, 1999.
- Schmidt, S., et al., "Watching the Growth of Bulk Grains During Recrystallization of Deformed Metals," *Science*, vol. 305, pp. 229-232, Jul. 9, 2004.
- Sumiya, Hitoshi, et al., "Synthesis of High-Purity Nano-Polycrystalline Diamond and Its Characterization," *SEI Technical Review*, No. 59, pp. 52-59, Jan. 2005.
- Wang, Guangzu, et al., "Effect of Recrystallized Graphite on the Nucleation of Diamond in Film Growth Reactions," *Science and Technology of New Diamond*, pp. 257-259, 1990.
- Wei, Xian-Wen, et al., "A solution phase fabrication of magnetic nanoparticles encapsulated in carbon," *Nanotechnology*, vol. 17, pp. 4307-4311, 2006.
- Welz, Sascha, et al., "Nucleation, growth, and graphitization of diamond nanocrystals during chlorination of carbides," *Journal of Applied Physics*, vol. 93, No. 7, pp. 4207-4214, Apr. 1, 2003.
- Wheeler, N.S., "Microstructural Characterization of Cobalt-Tungsten Coated Graphite Fibers," *J. Res. Natl. Inst. Stand. Technol.*, vol. 100, No. 6, pp. 641-659, Nov.-Dec. 1995.
- Wu, B.Y.C., et al., "Nanostructured Ni—Co Alloys with Tailorable Grain Size and Twin Density," *Metallurgical and Materials Transactions A*, vol. 36A, pp. 1927-1936, Jul. 2005.
- Yanchuk, I.B., et al., "Raman scattering, AFM and nanoindentation characterization of diamond films obtained by hot filament CVD," *Diamond and Related Materials*, vol. 12, pp. 266-269, 2004.
- Yushin, G.N., et al., "Effect of sintering on structure of nanodiamond," *Diamond and Related Materials*, vol. 14, pp. 1721-1729, 2005.
- Zhang, L., et al., "Ultrafine and nanoscaled tungsten carbide synthesis from colloidal carbon coated nano tungsten precursor," *Powder Metallurgy*, vol. 49, No. 4, pp. 369-373, 2006.
- Zhao, Y., et al., "Superhard B—C—N materials synthesized in nanostructured bulks," *J. Mater. Res.*, vol. 17, No. 12, pp. 3139-3145, Dec. 2002.

\* cited by examiner



**FIG. 1A**



**FIG. 1B**

**FIG. 2**

**FIG. 3**

**POLYCRYSTALLINE COMPACTS  
INCLUDING INTERBONDED  
NANOPARTICLES, CUTTING ELEMENTS  
AND EARTH-BORING TOOLS INCLUDING  
SUCH POLYCRYSTALLINE COMPACTS,  
AND RELATED METHODS**

**CROSS-REFERENCE TO RELATED  
APPLICATIONS**

This application is a continuation of U.S. patent application Ser. No. 13/226,127, filed Sep. 6, 2011, now U.S. Pat. No. 8,800,693, issued Aug. 12, 2014, which application claims the benefit of U.S. Provisional Patent Application Serial No. 61/411,355, filed Nov. 8, 2010, entitled "Polycrystalline Compacts Including Nanoparticulate Inclusions, Cutting Elements and Earth-Boring Tools Including Such Compacts, and Methods of Forming Same," the disclosure of each of which is incorporated herein in its entirety by this reference.

**TECHNICAL FIELD**

The present disclosure relates generally to polycrystalline compacts, which may be used, for example, as cutting elements for earth-boring tools, and to methods of forming such polycrystalline compacts, cutting elements, and earth-boring tools.

**BACKGROUND**

Earth-boring tools for forming wellbores in subterranean earth formations generally include a plurality of cutting elements secured to a body. For example, fixed-cutter earth-boring rotary drill bits (also referred to as "drag bits") include a plurality of cutting elements that are fixedly attached to a bit body of the drill bit. Similarly, roller cone earth-boring rotary drill bits may include cones that are mounted on bearing pins extending from legs of a bit body such that each cone is capable of rotating about the bearing pin on which it is mounted. A plurality of cutting elements may be mounted to each cone of the drill bit. In other words, earth-boring tools typically include a bit body to which cutting elements are attached.

The cutting elements used in such earth-boring tools often include polycrystalline diamond compacts (often referred to as "PDC"), which comprise a polycrystalline diamond material. Polycrystalline diamond material is material that includes interbonded grains or crystals of diamond material. In other words, polycrystalline diamond material includes direct, inter-granular bonds between the grains or crystals of diamond material. The terms "grain" and "crystal" are used synonymously and interchangeably herein.

Polycrystalline diamond compact cutting elements are typically formed by sintering and bonding together relatively small diamond grains under conditions of high temperature and high pressure in the presence of a catalyst (e.g., cobalt, iron, nickel, or alloys and mixtures thereof) to form a layer (e.g., a compact or "table") of polycrystalline diamond material on a cutting element substrate. These processes are often referred to as high temperature/high pressure (HTHP) processes. The cutting element substrate may comprise a cermet material (i.e., a ceramic-metal composite material) such as, for example, cobalt-cemented tungsten carbide. In such instances, the cobalt (or other catalyst material) in the cutting element substrate may be swept into the diamond grains during sintering and serve as the catalyst

material for forming the inter-granular diamond-to-diamond bonds, and the resulting diamond table, from the diamond grains. In other methods, powdered catalyst material may be mixed with the diamond grains prior to sintering the grains together in an HTHP process.

Upon formation of a diamond table using an HTHP process, catalyst material may remain in interstitial spaces between the grains of diamond in the resulting polycrystalline diamond compact. The presence of the catalyst material in the diamond table may contribute to thermal damage in the diamond table when the cutting element is heated during use, due to friction at the contact point between the cutting element and the formation.

Polycrystalline diamond compact cutting elements in which the catalyst material remains in the polycrystalline diamond compact are generally thermally stable up to a temperature of about seven hundred fifty degrees Celsius (750° C.), although internal stress within the cutting element may begin to develop at temperatures exceeding about three hundred fifty degrees Celsius (350° C.). This internal stress is at least partially due to differences in the rates of thermal expansion between the diamond table and the cutting element substrate to which it is bonded. This differential in thermal expansion rates may result in relatively large compressive and tensile stresses at the interface between the diamond table and the substrate, and may cause the diamond table to delaminate from the substrate. At temperatures of about seven hundred fifty degrees Celsius (750° C.) and above, stresses within the diamond table itself may increase significantly due to differences in the coefficients of thermal expansion of the diamond material and the catalyst material within the diamond table. For example, cobalt thermally expands significantly faster than diamond, which may cause cracks to form and propagate within the diamond table, eventually leading to deterioration of the diamond table and ineffectiveness of the cutting element.

Furthermore, at temperatures at or above about seven hundred fifty degrees Celsius (750° C.), some of the diamond crystals within the polycrystalline diamond compact may react with the catalyst material causing the diamond crystals to undergo a chemical breakdown or back-conversion to another allotrope of carbon or another carbon-based material. For example, the diamond crystals may graphitize at the diamond crystal boundaries, which may substantially weaken the diamond table. In addition, at extremely high temperatures, in addition to graphite, some of the diamond crystals may be converted to carbon monoxide and carbon dioxide.

In order to reduce the problems associated with differential rates of thermal expansion and chemical breakdown of the diamond crystals in polycrystalline diamond compact cutting elements, so-called "thermally stable" polycrystalline diamond compacts (which are also known as thermally stable products, or "TSPs") have been developed. Such a thermally stable polycrystalline diamond compact may be formed by leaching the catalyst material (e.g., cobalt) out from interstitial spaces between the interbonded diamond crystals in the diamond table using, for example, an acid or combination of acids (e.g., aqua regia). Substantially all of the catalyst material may be removed from the diamond table, or catalyst material may be removed from only a portion thereof. Thermally stable polycrystalline diamond compacts in which substantially all catalyst material has been leached out from the diamond table have been reported to be thermally stable up to temperatures of about twelve hundred degrees Celsius (1,200° C.). It has also been reported, however, that such fully leached diamond tables

are relatively more brittle and vulnerable to shear, compressive, and tensile stresses than are non-leached diamond tables. In addition, it is difficult to secure a completely leached diamond table to a supporting substrate. In an effort to provide cutting elements having polycrystalline diamond compacts that are more thermally stable relative to non-leached polycrystalline diamond compacts, but that are also relatively less brittle and vulnerable to shear, compressive, and tensile stresses relative to fully leached diamond tables, cutting elements have been provided that include a diamond table in which the catalyst material has been leached from a portion or portions of the diamond table. For example, it is known to leach catalyst material from a cutting face, from the side of the diamond table, or both, to a desired depth within the diamond table, but without leaching all of the catalyst material out from the diamond table.

#### BRIEF SUMMARY

In some embodiments, the present disclosure includes polycrystalline compacts that comprise a plurality of grains of hard material that are interbonded to form a polycrystalline hard material, and a plurality of particles disposed in interstitial spaces between the grains of hard material, the particles (e.g., nanoparticles) comprising a non-catalytic, non-carbide-forming metal. In some embodiments, the particles may comprise rhenium.

In additional embodiments, the present disclosure includes cutting elements and drill bits comprising at least one such polycrystalline compact.

In further embodiments, the present disclosure includes methods of forming polycrystalline compacts. The methods including forming a polycrystalline material including a hard material comprising a plurality of hard particles and a plurality of particles comprising a non-catalytic, non-carbide-forming material disposed in a plurality of interstitial spaces between a plurality of interbonded grains of the hard material.

In yet further embodiments, the present disclosure includes methods of forming polycrystalline compacts, in which a plurality of hard particles and a plurality of non-catalytic, non-carbide-forming particles (e.g., nanoparticles) are sintered to form a polycrystalline hard material comprising a plurality of interbonded grains of hard material.

In additional embodiments, the present disclosure includes methods of forming cutting elements in which interstitial spaces between interbonded grains of hard material in a polycrystalline material are infiltrated with a plurality of non-catalytic, non-carbide-forming particles (e.g., nanoparticles).

#### BRIEF DESCRIPTION OF THE DRAWINGS

While the specification concludes with claims particularly pointing out and distinctly claiming what are regarded as embodiments of the present disclosure, various features and advantages of embodiments of the disclosure may be more readily ascertained from the following description of some embodiments of the disclosure when read in conjunction with the accompanying drawings, in which:

FIG. 1A is a partial cut-away perspective view illustrating an embodiment of a cutting element comprising a polycrystalline compact of the present disclosure;

FIG. 1B is a simplified drawing showing how a microstructure of the polycrystalline compact of FIG. 1A may appear under magnification, and illustrates interbonded and interspersed larger and smaller grains of hard material;

FIG. 2 includes an enlarged view of one embodiment of a non-catalytic, non-carbide-forming nanoparticle of the present disclosure; and

FIG. 3 is a perspective view of an embodiment of a fixed-cutter earth-boring rotary drill bit that includes a plurality of polycrystalline compacts like that shown in FIGS. 1A and 1B.

#### DETAILED DESCRIPTION

The illustrations presented herein are not actual views of any particular polycrystalline compact, microstructure of a polycrystalline compact, particle, cutting element, or drill bit, and are not drawn to scale, but are merely idealized representations employed to describe the present disclosure. Additionally, elements common between figures may retain the same numerical designation.

As used herein, the term "drill bit" means and includes any type of bit or tool used for drilling during the formation or enlargement of a wellbore and includes, for example, rotary drill bits, percussion bits, core bits, eccentric bits, bi-center bits, reamers, mills, drag bits, roller cone bits, hybrid bits and other drilling bits and tools known in the art.

As used herein, the term "nanoparticle" means and includes any particle or grain of material having an average particle diameter of about 500 nm or less. Nanoparticles include grains in a polycrystalline material having an average grain size of about 500 nm or less.

As used herein, the term "polycrystalline material" means and includes any material comprising a plurality of grains or crystals of the material that are bonded directly together by inter-granular bonds. The crystal structures of the individual grains of the material may be randomly oriented in space within the polycrystalline material.

As used herein, the term "polycrystalline compact" means and includes any structure comprising a polycrystalline material formed by a process that involves application of pressure (e.g., compaction) to the precursor material or materials used to form the polycrystalline material.

As used herein, the term "inter-granular bond" means and includes any direct atomic bond (e.g., covalent, metallic, etc.) between atoms in adjacent grains of material.

As used herein, the term "catalyst material" refers to any material that is capable of substantially catalyzing the formation of inter-granular bonds between grains of hard material during a sintering process (e.g., an HTHP process). For example, catalyst materials for diamond include cobalt, iron, nickel, other elements from Group VIIA of the Periodic Table of the Elements, and alloys thereof.

As used herein, the term "non-catalytic material" refers to any material that is at least substantially not a catalyst material.

As used herein, the term "hard material" means and includes any material or particles thereof having a Knoop hardness value of about 2,000 Kg/mm<sup>2</sup> (20 GPa) or more. In some embodiments, the hard materials employed herein may have a Knoop hardness value of about 3,000 Kg/mm<sup>2</sup> (29.4 GPa) or more. Such materials include, for example, diamond and cubic boron nitride.

As used herein, the term "non-catalytic, non-carbide-forming nanoparticle" means and includes any nanoparticle that is not comprised of a catalyst material, diamond, or cubic boron nitride, and that is at least substantially unreactive with carbon at conditions commonly achieved during formation and use of a polycrystalline table. Substantially non-catalytic, non-carbide-forming nanoparticles, in some embodiments, may comprise refractory metals and alloys

thereof as described in greater detail below. In some embodiments, the non-catalytic, non-carbide-forming nanoparticles may also be at least substantially unreactive with a catalyst material.

FIG. 1A is a simplified, partially cut-away perspective view of an embodiment of a cutting element 10 of the present disclosure. The cutting element 10 comprises a polycrystalline compact in the form of a layer of hard polycrystalline material 12, also known in the art as a polycrystalline table, that is provided on (e.g., formed on or attached to) a supporting substrate 16 with an interface 14 therebetween. Though the cutting element 10 in the embodiment depicted in FIG. 1A is cylindrical or disc-shaped, in other embodiments, the cutting element 10 may have any desirable shape, such as a dome, cone, chisel, etc.

In some embodiments, the polycrystalline material 12 comprises polycrystalline diamond. In such embodiments, the cutting element 10 may be referred to as a polycrystalline diamond compact (PDC) cutting element. In other embodiments, the polycrystalline material 12 may comprise another hard material such as, for example, polycrystalline cubic boron nitride.

FIG. 1B is an enlarged view illustrating how a microstructure of the polycrystalline material 12 of the cutting element 10 may appear under magnification. As discussed in further detail below, the polycrystalline material 12 includes interbonded grains 18 of hard material. The polycrystalline material 12 also includes particles 19 (e.g., nanoparticles) disposed in interstitial spaces 22 between the interbonded grains 18 of hard material. These particles 19 in the polycrystalline material 12 may reduce an amount of catalyst material remaining in the polycrystalline material 12 as a catalyst material is used to catalyze formation of the polycrystalline material 12 in a sintering process, such as a high temperature, high pressure (HTHP) process. In other words, at least substantially non-catalytic, non-carbide-forming particulate inclusions (i.e., particles 19) may be incorporated into the polycrystalline material 12 such that the amount of catalyst material remaining in interstitial spaces 22 between the interbonded grains 18 of hard material in the microstructure after the sintering process is reduced by volumetric exclusion based on the presence of the non-catalyst, non-carbide-forming particles 19. The spatial volume occupied by these particles 19 cannot be occupied by catalyst material, and, hence, the amount of catalyst material in the polycrystalline material 12 is reduced. The overall reduction of catalytic material in the grain boundary regions between the interbonded grains 18 of hard material may lead to an increase in thermal stability of the cutting element 10 by having a reduced coefficient of thermal expansion mismatch effect from the reduced content of catalyst material. Furthermore, in embodiments in which the hard material comprises diamond, the reduction of catalytic material in between the interbonded grains 18 of hard material may also decrease the susceptibility of the diamond to graphitize (often referred to as "reverse graphitization") for substantially the same reasons.

The particles 19 in the polycrystalline material 12 may also lower an overall thermal conductivity of the polycrystalline material 12. In other words, the particulate inclusions (i.e., particles 19) may have a lower thermal conductivity than at least the interbonded grains 18 of hard material such that the overall thermal conductivity of the polycrystalline material 12 is reduced.

The overall reduction of thermal conductivity in the polycrystalline material 12 may lead to an increase in thermal stability of the cutting element 10. The particles 19

having a low thermal conductivity may act to insulate or slow the distribution of heat to at least a portion of the polycrystalline material 12. For example, during drilling of an earth formation, a temperature of an exterior of the polycrystalline material 12 may increase due to frictional forces between the polycrystalline material 12 and the earth formation. Because of the reduced overall thermal conductivity of the polycrystalline material 12, the increased temperature may be at least partially contained to the exterior of the polycrystalline material 12. This may help to maintain an interior portion of the polycrystalline material 12 at a lower and more stable temperature. Accordingly, by insulating at least a portion of the polycrystalline material 12, the insulated portion of the polycrystalline material may be relatively less likely to degrade during use due to thermal expansion mismatch between the different elements within the polycrystalline material. Furthermore, in embodiments in which the hard material comprises diamond, the reduction of heat transferred to at least a portion of the polycrystalline material 12 may also decrease the susceptibility of the diamond to graphitize (often referred to as "reverse graphitization").

In some embodiments, the grains 18 of hard material in the polycrystalline material 12 may have a uniform, mono-modal grain size distribution, as shown in FIG. 1B.

In additional embodiments, the grains 18 of the polycrystalline material 12 may have a multi-modal (e.g., bi-modal, tri-modal, etc.) grain size distribution. For example, the polycrystalline material 12 may comprise a multi-modal grain size distribution as disclosed in at least one of Provisional U.S. Patent Application Ser. No. 61/232,265, which was filed on Aug. 7, 2009, and entitled "Polycrystalline Compacts Including In-Situ Nucleated Grains, Earth-Boring Tools Including Such Compacts, and Methods Of Forming Such Compacts and Tools," and U.S. patent application Ser. No. 12/558,184, which was filed on Sep. 11, 2009, now U.S. Pat. No. 8,727,042, issued May 20, 2014, and entitled "Polycrystalline Compacts Having Material Disposed In Interstitial Spaces Therein, And Cutting Elements Including Such Compacts," the disclosure of each of which is incorporated herein in its entirety by this reference.

As known in the art, the average grain size of grains within a microstructure may be determined by measuring grains of the microstructure under magnification. For example, a scanning electron microscope (SEM), a field emission scanning electron microscope (FESEM), or a transmission electron microscope (TEM) may be used to view or image a surface of a polycrystalline material 12 (e.g., a polished and etched surface of the polycrystalline material 12). Commercially available vision systems are often used with such microscopy systems, and these vision systems are capable of measuring the average grain size of grains within a microstructure.

In some embodiments, at least some of the grains 18 of hard material may comprise in-situ nucleated grains 18 of hard material, as disclosed in the aforementioned provisional U.S. Patent Application Ser. No. 61/232,265, which was filed on Aug. 7, 2009.

The interstitial spaces 22 between the grains 18 of hard material may be at least partially filled with non-catalytic, non-carbide-forming particles 19 (e.g., nanoparticles) and with a catalyst material 24.

The particles 19 disposed in the interstitial spaces 22 between the interbonded grains 18 of hard material may comprise a non-catalytic, non-carbide-forming material. The non-catalytic, non-carbide-forming material of the particles 19 may comprise, for example, a refractory metal. As particular non-limiting examples, the non-catalytic, non-

carbide-forming particles **19** may comprise at least one of rhenium, osmium, ruthenium, rhodium, iridium, platinum, molybdenum, and alloys thereof.

In additional embodiments, the material of the non-catalytic, non-carbide-forming particles **19** may be selected such that at least a portion of the particles **19** do not react with the catalyst material **24** or may only form a solid solution between the materials. For example, in one embodiment, the particles **19** may comprise at least one of rhenium, platinum, and ruthenium, and the catalyst material **24** may comprise cobalt. Rhenium, for example, is believed to be at least substantially unreactive with cobalt at temperatures, pressures, and durations of sintering processes used in the formation of the polycrystalline material **12** as described in greater detail below.

Because at least a portion of the particles **19** may not react with the catalyst material **24** or may only form a solid solution, the particles **19** may help to lower an overall thermal conductivity of the polycrystalline material **12**. For example, the particles **19** may have a thermal conductivity less than a thermal conductivity of the catalyst material **24**. In some embodiments, the particles **19** may have a thermal conductivity of about three quarters or less of a thermal conductivity of the catalyst material **24**. For example, in one embodiment, the particles **19** may comprise rhenium which has a thermal conductivity of about forty-eight watts per meter-Kelvin ( $48 \text{ Wm}^{-1}\text{K}^{-1}$ ) and the catalyst material **24** may comprise cobalt which has a thermal conductivity of about one hundred watts per meter-Kelvin ( $100 \text{ Wm}^{-1}\text{K}^{-1}$ ). Additionally, because at least a portion of the particles **19** may not react with the catalyst material **24**, the particles **19** may help to reduce the variations in linear coefficients of thermal expansion throughout the polycrystalline material. For example, the particles **19** may have a linear coefficient of thermal expansion less than a linear coefficient of thermal expansion of the catalyst material **24**. In some embodiments, the particles **19** may have a linear coefficient of thermal expansion of about one-half or less of the linear coefficient of thermal expansion of the catalyst material **24**. For example, in one embodiment, the particles **19** may comprise rhenium which has a linear coefficient of thermal expansion of about  $6.2 \times 10^{-6} \text{ K}^{-1}$  and the catalyst material **24** may comprise cobalt which has a linear coefficient of thermal expansion of about  $13.0 \times 10^{-6} \text{ K}^{-1}$ . In some embodiments, material of the particles **19** may have a zero or negative linear coefficient of thermal expansion. In other words, material of the particles **19** may be selected to exhibit substantially no expansion or contraction when subjected to heating. For example, the particles **19** may comprise zirconium tungstate that exhibits a negative linear coefficient of thermal expansion.

In some embodiments, the non-catalytic, non-carbide-forming particles **19** may, at least initially (prior to a sintering process used to form the polycrystalline material **12**), comprise at least two materials, as does a particle **100** illustrated in FIG. 2. In some embodiments, the particle **100** may comprise a nanoparticle. For example, the particle **100** may include a core **102** comprising a first material and one or more coatings **104**, **106**, **108** comprising at least one other material. For example, at least one of the core **102** and the one or more coatings **104**, **106**, **108** comprises a non-catalytic, non-carbide-forming material while another portion of the particle comprised another material (e.g., an oxide, a carbide, a refractory metal, a catalytic metal, an alloy, a cermet, a ceramic, a clay, a mineral, a fullerene, a carbon nanotube (CNT), a graphene, combinations thereof, etc.). In some embodiments, the core **102** may comprise the

catalyst material **24**. In some embodiments, at least one coating **104**, **106**, **108** may comprise the catalyst material **24** while at least one other coating **104**, **106**, **108** comprises a non-catalytic, non-carbide-forming material.

The core **102** may comprise a single nanoparticle or the core may comprise a plurality or cluster of smaller nanoparticles **103**. The core **102**, comprising one particle or a plurality of particles **103**, may have a total average particle size of between about twenty-five nanometers (25 nm) and about seventy-five nanometers (75 nm). For example, in one embodiment, the core **102** may comprise a single particle of cobalt having an average particle size of about twenty-five nanometers (25 nm). In another embodiment, the core **102** may comprise a plurality of nanoparticles **103** having an average particle size of about two nanometers (2 nm) to about ten nanometers (10 nm) which have agglomerated to form the core **102** having an average particle size of about fifty nanometers (50 nm) to about seventy-five nanometers (75 nm). The plurality of nanoparticles **103** may have a uniform average particle size or the plurality of nanoparticles **103** may have differing average particle sizes. In yet further embodiments, the plurality of nanoparticles **103** forming the core **102** may comprise at least two materials. For example, in one embodiment, at least one nanoparticle of the plurality of nanoparticles **103** may comprise cobalt and at least one nanoparticle of the plurality of nanoparticles **103** may comprise a non-catalytic, non-carbide-forming material such as rhenium, platinum, osmium, or an alloy or mixture thereof.

In some embodiments, the one or more coatings **104**, **106**, **108** of the particles **100** may comprise rhenium. For example, the particles **100** may comprise a core **102** comprising one or more nanoparticles **103** of diamond and one or more coatings **104**, **106**, **108** comprising rhenium. By way of further example, the particles **100** may comprise a core **102** comprising one or more nanoparticles **103** of zirconium tungstate and one or more coatings **104**, **106**, **108** comprising rhenium. By way of yet further example, the particles **100** may comprise a core **102** comprising one or more nanoparticles **103** of scandium tungstate and one or more coatings **104**, **106**, **108** comprising rhenium.

In additional embodiments, the one or more coatings **104**, **106**, **108** of the particles **100** may comprise molybdenum. For example, the particles **100** may comprise a core **102** comprising one or more nanoparticles **103** of diamond and one or more coatings **104**, **106**, **108** comprising molybdenum. By way of further example, the particles **100** may comprise a core **102** comprising one or more nanoparticles **103** of zirconium tungstate and one or more coatings **104**, **106**, **108** comprising molybdenum.

Each coating of the one or more coatings **104**, **106**, **108** may have a thickness of between about two nanometers (2 nm) and about five nanometers (5 nm). In some embodiments each of the at least one coating **104**, **106**, **108** may be conformally deposited on the core **102**. In some embodiments, multiple coatings of the same material may be formed over the core **102**. For example, a first coating **104**, a second coating **106**, and a third coating **108** each comprising rhenium may be formed over the core **102**. In alternative embodiments, at least two coatings **104**, **106**, **108** comprising different materials may be formed on the core **102**. For example, in one embodiment the first coating **104** comprising rhenium may be formed over the core **102**, the second coating **106** comprising platinum may be formed over the first coating **104**, and the third coating **108** comprising rhenium may be formed over the second coating **106**. While FIG. 2 is illustrated as having three coatings **104**, **106**,

**108** over the core **102**, it is understood that any number of coatings may be applied to the core **102** such that the total particle comprises a nanoparticle. In further embodiments, micron sized clusters formed of at least two nanoparticles, like the particle **100** of FIG. 2, may be conglomerated and coated either individually or in combination and incorporated into the polycrystalline material **12**.

By way of example and not limitation, processes (e.g., nanoencapsulation process) such as liquid sol-gel, flame spray pyrolysis, chemical vapor deposition (CVD), physical vapor deposition (PVD) (e.g., sputtering), and atomic layer deposition (ALD), may be used to provide the one or more coatings **104**, **106**, **108** on the core **102**. Other techniques that may be used to provide the at least one coating **104**, **106**, **108** on the core **102** include colloidal coating processes, plasma coating processes, microwave plasma coating processes, physical admixture processes, van der Waals coating processes, and electrophoretic coating processes. In some embodiments, the one or more coatings **104**, **106**, **108** may be provided on the core **102** in a fluidized bed reactor.

Referring again to FIGS. 1A and 1B, the volume occupied by the particles **19** in the polycrystalline material **12** may be in a range extending from about 0.01% to about 50% of the volume of the polycrystalline material **12**. The weight percentage of the particles **19** in the polycrystalline material **12** may be in a range extending from about 0.1% to about 10% by weight.

In some embodiments, as least some of the non-catalytic, non-carbide-forming particles **19** may be bonded to the grains **18** of hard material after the sintering process (e.g., an HPHT process) used to form the polycrystalline material **12**.

In some embodiments, the polycrystalline material **12** may also include the catalyst material **24** disposed in interstitial spaces **22** between the interbonded grains **18** of the polycrystalline hard material and between the particles **19**. The catalyst material **24** may comprise a catalyst used to catalyze the formation of inter-granular bonds **26** between the grains **18** of hard material in the polycrystalline material **12**. In other embodiments, however, the interstitial spaces **22** between the grains **18** and the particles **19** in some or all regions of the polycrystalline material **12** may be at least substantially free of such a catalyst material **24**. In such embodiments, the interstitial spaces **22** may comprise voids filled with gas (e.g., air).

In embodiments in which the polycrystalline material **12** comprises polycrystalline diamond, the catalyst material **24** may comprise a Group VIIIA element (e.g., iron, cobalt, or nickel) or an alloy thereof, and the catalyst material **24** may comprise between about one half of one percent (0.1%) and about ten percent (10%) by volume of the hard polycrystalline material **12**. In additional embodiments, the catalyst material **24** may comprise a carbonate material such as, for example, a carbonate of one or more of magnesium, calcium, strontium, and barium. Carbonates may also be used to catalyze the formation of polycrystalline diamond.

The layer of hard polycrystalline material **12** of the cutting element **10** may be formed using a high temperature/high pressure (HTHP) process. Such processes, and systems for carrying out such processes, are generally known in the art. In some embodiments, the polycrystalline material **12** may be formed on a supporting substrate **16** (as shown in FIG. 1A) of cemented tungsten carbide or another suitable substrate material in a conventional HTHP process of the type described, by way of non-limiting example, in U.S. Pat. No. 3,745,623 to Wentorf et al. (issued Jul. 17, 1973), or may be formed as a freestanding polycrystalline material **12** (i.e., without the supporting substrate **16**) in a similar

conventional HTHP process as described, by way of non-limiting example, in U.S. Pat. No. 5,127,923 Bunting et al. (issued Jul. 7, 1992), the disclosure of each of which patents is incorporated herein in its entirety by this reference. In some embodiments, the catalyst material **24** may be supplied from the supporting substrate **16** during an HTHP process used to form the polycrystalline material **12**. For example, the substrate **16** may comprise a cobalt-cemented tungsten carbide material. The cobalt of the cobalt-cemented tungsten carbide may serve as the catalyst material **24** during the HTHP process. Furthermore, in some embodiments, the particles **19** also may be supplied from the supporting substrate **16** during an HTHP process used to form the polycrystalline material **12**. For example, the substrate **16** may comprise a cobalt-cemented tungsten carbide material that also includes particles **19** therein. The particles **19** of the substrate may sweep into the interstitial spaces **22** between the grains **18** of hard material.

To form the polycrystalline material **12** in an HTHP process, a particulate mixture comprising particles (e.g., grains) of hard material and non-catalytic, non-carbide-forming particles **100** (e.g., nanoparticles **100**) may be subjected to elevated temperatures (e.g., temperatures greater than about one thousand degrees Celsius (1,000° C.)) and elevated pressures (e.g., pressures greater than about five gigapascals (5.0 GPa)) to form inter-granular bonds **26** between the particles of hard material and the particles **100**, thereby forming the interbonded grains **18** of hard material and the particles **19** of the polycrystalline material **12**. In some embodiments, the particulate mixture may be subjected to a pressure greater than about six gigapascals (6.0 GPa) and a temperature greater than about one thousand five hundred degrees Celsius (1,500° C.) in the HTHP process.

Because it may be desirable to keep at least a portion of the particles **19** unreacted with the catalyst material **24**, in some embodiments, the polycrystalline material **12** may be formed in more than one HTHP process or cycle wherein each HTHP process has a limited temperature, pressure, and duration. For example, each HTHP process may be for less than about two minutes and at temperatures lower than about 1,500° C. By limiting the duration of the each HTHP process, a diffusion of the catalyst material **24** into the particles **19** may be limited thereby maintaining the integrity of at least a portion of the particles **19**.

The particulate mixture may comprise hard particles for forming the grains **18** of hard material previously described herein. The particulate mixture may also comprise at least one of particles of catalyst material **24**, and non-catalytic, non-carbide-forming particles (e.g., nanoparticles), such as particles **100** as previously described with reference to FIG. 2 or particles at least substantially comprised of a non-catalytic, non-carbide-forming material for forming the particles **19** in the polycrystalline material **12**. In some embodiments, the particulate mixture may comprise a powder-like substance. In other embodiments, however, the particulate mixture may be carried by (e.g., on or in) another material, such as a paper or film, which may be subjected to the HTHP process. An organic binder material also may be included with the particulate mixture to facilitate processing.

Thus, in some embodiments, the non-catalytic, non-carbide-forming particles (e.g., particles **100**) may be admixed with the hard particles used to form the grains **18** to form a particulate mixture, which then may be sintered in an HPHT process.

In some embodiments, the non-catalytic, non-carbide-forming particles (e.g., particles **100**) may be admixed with the hard particles used to form the grains **18** of hard material

## 11

prior to a modified HPHT sintering process used to synthesize a nanoparticulate composite that includes the non-catalytic, non-carbide-forming particles and nanoparticles of hard material.

In some embodiments, the non-catalytic, non-carbide-forming particles may be grown on, attached, adhered, or otherwise connected to the hard particles used to form the grains **18** prior to the sintering process. The non-catalytic, non-carbide-forming particles may be attached to the hard particles by functionalizing exterior surfaces of at least one of the non-catalytic, non-carbide-forming particles and the hard particles. After attaching the non-catalytic, non-carbide-forming particles to the hard particles, the resulting particulate mixture may be subjected to an HPHT process to form a polycrystalline material **12** comprising grains of hard material **19** and non-catalytic, non-carbide-forming particles **19**, as described above.

In additional embodiments, the non-catalytic, non-carbide-forming particles may be combined with the catalyst material prior to the sintering process. For example, the non-catalytic, non-carbide-forming particles may be grown on, attached, adhered, or otherwise connected to particles of catalyst material, and the coated particles of catalyst material may be combined with hard particles to form the particulate mixture prior to the sintering process. The non-catalytic, non-carbide-forming particles may be attached to the particles of catalyst material by functionalizing exterior surfaces of at least one of the non-catalytic, non-carbide-forming particles and the catalyst particles. After attaching the non-catalytic, non-carbide-forming particles to the catalyst particles and admixing with hard particles, the resulting particulate mixture may be subjected to an HPHT process to form a polycrystalline material **12**, as described above.

In some embodiments, the non-catalytic, non-carbide-forming particles may be grown on, attached, adhered, or otherwise connected to both particles of hard material and particles of catalyst material, and the coated particles may be combined to form the particulate mixture.

As previously mentioned, a particulate mixture that includes hard particles for forming the interbonded grains **18** of hard material, non-catalytic, non-carbide-forming particles, and, optionally, a catalyst material **24** (for catalyzing the formation of inter-granular bonds **26** between the grains **18**), may be subjected to an HTHP process to form a polycrystalline material **12**. After the HTHP process, catalyst material **24** (e.g., cobalt) and non-catalytic, non-carbide-forming particles **19** may be disposed in at least some of the interstitial spaces **22** between the interbonded grains **18** of hard material.

Optionally, the catalyst material **24** may be removed from the polycrystalline material **12** after the HTHP process using processes known in the art. However, the removal of said catalyst material **24** may also result in the removal of at least a portion of the non-catalytic, non-carbide-forming particles **19**, which may be undesirable. For example, a leaching process may be used to remove the catalyst material **24** and/or the non-catalytic, non-carbide-forming particles **19** from the interstitial spaces **22** between the grains **18** of hard material in at least a portion of the polycrystalline material **12**. By way of example and not limitation, a portion of the polycrystalline material **12** may be leached using a leaching agent and process such as those described more fully in, for example, U.S. Pat. No. 5,127,923 to Bunting et al. (issued Jul. 7, 1992), and U.S. Pat. No. 4,224,380 to Bovenkerk et al. (issued Sep. 23, 1980), the disclosure of each of which patent is incorporated herein in its entirety by this reference. Specifically, aqua regia (a mixture of concentrated nitric acid

## 12

( $\text{HNO}_3$ ) and concentrated hydrochloric acid (HCl)) may be used to at least substantially remove catalyst material **24** and/or non-catalytic, non-carbide-forming nanoparticles from the interstitial spaces **22**. It is also known to use boiling hydrochloric acid (HCl) and boiling hydrofluoric acid (HF) as leaching agents. One particularly suitable leaching agent is hydrochloric acid (HCl) at a temperature of above one hundred ten degrees Celsius ( $110^\circ \text{ C.}$ ), which may be provided in contact with the polycrystalline material **12** for a period of about two (2) hours to about sixty (60) hours, depending upon the size of the body of polycrystalline material **12**. After leaching the polycrystalline material **12**, the interstitial spaces **22** between the interbonded grains **18** of hard material within the polycrystalline material **12** subjected to the leaching process may be at least substantially free of catalyst material **24** used to catalyze formation of inter-granular bonds **26** between the grains in the polycrystalline material **12**. Only a portion of the polycrystalline material **12** may be subjected to the leaching process, or the entire body of the polycrystalline material **12** may be subjected to the leaching process.

In additional embodiments of the present disclosure, non-catalytic, non-carbide-forming particles **19**, **100** may be introduced into the interstitial spaces **22** between interbonded grains **18** of hard, polycrystalline material **12** after catalyst material **24** and any other material in the interstitial spaces **22** has been removed from the interstitial spaces **22** (e.g., by a leaching process). For example, after subjecting a polycrystalline material **12** to a leaching process, non-catalytic, non-carbide-forming particles **19**, **100** may be introduced into the interstitial spaces **22** between the grains **18** of hard material in the polycrystalline material **12**. Non-catalytic, non-carbide-forming particles **19**, **100** may be suspended in a liquid (e.g., water or another polar solvent) to form a suspension, and the leached polycrystalline material **12** may be soaked in the suspension to allow the liquid and the non-catalytic, non-carbide-forming particles **19**, **100** to infiltrate into the interstitial spaces **22**. The liquid (and the non-catalytic, non-carbide-forming particles **19**, **100** suspended therein) may be drawn into the interstitial spaces **22** by capillary forces. In some embodiments, pressure may be applied to the liquid to facilitate infiltration of the liquid suspension into the interstitial spaces **22**.

After infiltrating the interstitial spaces **22** with the liquid suspension, the polycrystalline material **12** may be dried to remove the liquid from the interstitial spaces **22**, leaving behind the non-catalytic, non-carbide-forming particles **19**, **100** therein. Optionally, a thermal treatment process may be used to facilitate the drying process.

The polycrystalline material **12** then may be subjected to a thermal process (e.g., a standard vacuum furnace sintering process) to at least partially sinter the non-catalytic, non-carbide-forming particles **19**, **100** within the interstitial spaces **22** in the polycrystalline material **12**. Such a process may be carried out below any temperature that might be detrimental to the polycrystalline material **12**.

Embodiments of cutting elements **10** of the present disclosure that include a polycrystalline compact comprising polycrystalline material **12** formed as previously described herein, such as the cutting element **10** illustrated in FIG. 1A, may be formed and secured to an earth-boring tool such as, for example, a rotary drill bit, a percussion bit, a coring bit, an eccentric bit, a reamer tool, a milling tool, etc., for use in forming wellbores in subterranean formations. As a non-limiting example, FIG. 3 illustrates a fixed cutter type earth-boring rotary drill bit **36** that includes a plurality of cutting elements **10**, each of which includes a polycrystal-

## 13

line compact comprising polycrystalline material 12 as previously described herein. The rotary drill bit 36 includes a bit body 38, and the cutting elements 10, which include polycrystalline compacts 12, are bonded to the bit body 38. The cutting elements 10 may be brazed (or otherwise secured) within pockets formed in the outer surface of the bit body 38.

In some embodiments, the polycrystalline material 12 may be formed as a multi-portion polycrystalline material as described in, for example, provisional U.S. Patent Application Ser. No. 61/373,617, filed Aug. 13, 2010 and entitled "Cutting Elements Including Nanoparticles in At Least One Portion Thereof, Earth-Boring Tools Including Such Cutting Elements, and Related Methods," the disclosure of which is incorporated herein in its entirety by this reference.

Polycrystalline hard materials that include non-catalytic, non-carbide-forming nanoparticles in interstitial spaces between the interbonded grains of hard material, as described hereinabove, may exhibit improved thermal stability, improved mechanical durability, or both improved thermal stability and improved mechanical durability relative to previously known polycrystalline hard materials. By including the non-catalytic, non-carbide-forming nanoparticles in the interstitial spaces between the interbonded grains of hard material, less catalyst material may be disposed in interstitial spaces between the grains in the ultimate polycrystalline hard material, and the thermal conductivity of the polycrystalline material may be reduced, which may improve one or both of the thermal stability and the mechanical durability of the polycrystalline hard material.

The foregoing description is directed to particular embodiments for the purpose of illustration and explanation. It will be apparent, however, to one skilled in the art that many modifications and changes to the embodiments set forth above are possible without departing from the scope of the embodiments disclosed herein as hereinafter claimed, including legal equivalents. It is intended that the following claims be interpreted to embrace all such modifications and changes.

Additional non-limiting example Embodiments are described below.

Embodiment 1: A polycrystalline compact, comprising: a plurality of grains of hard material, the plurality of grains of hard material being interbonded to form a polycrystalline hard material; and a plurality of particles disposed in interstitial spaces between the grains of hard material, the plurality of particles comprising a non-catalytic, non-carbide-forming material.

Embodiment 2: The polycrystalline compact of Embodiment 1, wherein the plurality of grains of hard material comprises grains of diamond.

Embodiment 3: The polycrystalline compact of Embodiment 1 or Embodiment 2, wherein the particles comprise a refractory metal.

Embodiment 4: The polycrystalline compact of Embodiment 1 or Embodiment 2, wherein the particles comprise at least one of rhenium, osmium, ruthenium, rhodium, iridium, and platinum.

Embodiment 5: The polycrystalline compact of any one of Embodiments 1 through 4, further comprising a catalyst material in the interstitial spaces between the grains of hard material.

Embodiment 6: The polycrystalline compact of any one of Embodiments 1 through 5, wherein the particles comprise a material having a lower thermal conductivity than a thermal conductivity of the catalyst material.

## 14

Embodiment 7: The polycrystalline compact of Embodiment 5, wherein the particles comprise a material having a lower coefficient of thermal expansion than a coefficient of thermal expansion of the catalyst material.

Embodiment 8: The polycrystalline compact of any one of Embodiment 1 through 7, wherein the particles of the plurality of particles comprise: a core comprising a first material; and at least one coating on the core, the at least one coating comprising a second, different material.

Embodiment 9: The polycrystalline compact of Embodiment 8, wherein the core comprises at least two particles.

Embodiment 10: The polycrystalline compact of Embodiment 8, wherein the core comprises cobalt and the at least one coating on the core comprises rhenium.

Embodiment 11: The polycrystalline compact of Embodiment 8, wherein the at least one coating on the core comprises a first coating comprising rhenium, a second coating comprising platinum, and a third coating comprising rhenium.

Embodiment 12: The polycrystalline compact of any one of Embodiments 1 through 11, wherein the particles of the plurality of particles are about 0.01% to about 50% by volume of the polycrystalline compact.

Embodiment 13: A cutting element, comprising: a substrate; and a polycrystalline compact as recited in any one of Embodiments 1 through 12 on the substrate.

Embodiment 14: An earth-boring tool comprising a polycrystalline compact as recited in any one of Embodiments 1 through 12.

Embodiment 15: The earth-boring tool of Embodiment 14, wherein the earth-boring tool is a fixed-cutter rotary drill bit.

Embodiment 16: A method of forming a polycrystalline compact, comprising sintering a plurality of hard particles and a plurality of particles to form a polycrystalline hard material comprising a plurality of interbonded grains of hard material, the particles comprising a non-catalytic, non-carbide-forming material.

Embodiment 17: The method of Embodiment 16, further comprising selecting each of the hard particles of the plurality of hard particles to comprise diamond.

Embodiment 18: The method of Embodiment 16 or Embodiment 17, further comprising selecting the particles of the plurality of particles to a refractory metal.

Embodiment 19: The method of Embodiment 16 through 18, further comprising selecting the particles of the plurality of particles to comprise rhenium.

Embodiment 20: The method of any one of Embodiment 16 through 19, further comprising catalyzing the formation of inter-granular bonds between the grains of hard material.

Embodiment 21: The method of any one of Embodiments 16 through 20, wherein sintering a plurality of hard particles and a plurality of particles comprises sintering the plurality of hard particles and the plurality of particles in at least two HTHP processes, each process of the at least two HTHP processes being less than about two minutes in duration.

Embodiment 22: The method of any one of Embodiments 16 through 21, further comprising forming a particle of the plurality of particles comprising: coating a core comprising a first material with a second material, the second material comprising the non-catalytic, non-carbide-forming material.

Embodiment 23: A method of forming a cutting element, comprising infiltrating interstitial spaces between interbonded grains of hard material in a polycrystalline material with a plurality of particles, the particles comprising a non-catalytic, non-carbide-forming material.

## 15

Embodiment 24: The method of Embodiment 23, further comprising selecting the grains of hard material to comprise diamond grains.

Embodiment 25: The method of Embodiment 23 or Embodiment 24, further comprising selecting the particles of the plurality of particles to comprise a refractory metal.

Embodiment 26: The method of any one of Embodiments 23 through 25, further comprising selecting the particles of the plurality of particles to comprise at least one of rhenium, osmium, ruthenium, rhodium, iridium, platinum.

What is claimed is:

1. A polycrystalline compact, comprising:  
a polycrystalline hard material comprising interbonded

grains of hard material; and  
interbonded nanoparticles of non-carbide-forming mate-  
rial within interstitial spaces between the interbonded  
grains of the hard material, at least a portion of the  
interbonded nanoparticles of non-carbide-forming  
material interbonded with the interbonded grains of  
hard material.

2. The polycrystalline compact of claim 1, further comprising at least one of cobalt, nickel, and iron at least partially surrounding the interbonded nanoparticles of non-carbide-forming material within at least a portion of the interstitial spaces.

3. The polycrystalline compact of claim 2, wherein the at least one of cobalt, nickel, and iron is substantially absent from a portion of the polycrystalline hard material.

4. The polycrystalline compact of claim 1, wherein substantially all of the interstitial spaces are substantially free of cobalt, nickel, and iron.

5. The polycrystalline compact of claim 1, wherein the polycrystalline hard material comprises diamond.

6. The polycrystalline compact of claim 1, wherein the interbonded nanoparticles of non-carbide-forming material comprise one or more of elemental rhenium, elemental molybdenum, elemental osmium, elemental ruthenium, elemental rhodium, elemental iridium, elemental platinum, alloys thereof, scandium tungstate, and zirconium tungstate.

7. A cutting element, comprising:  
a substrate; and  
the polycrystalline compact of claim 1 over and attached  
to the substrate.

8. An earth-boring tool, comprising:  
a body; and  
cutting elements carried by the body, at least one of the  
cutting elements comprising the polycrystalline com-  
pact of claim 1.

9. A polycrystalline compact, comprising:  
a polycrystalline hard material comprising interbonded  
grains of hard material; and  
interbonded nanoparticles of non-carbide-forming mate-  
rial comprising rhenium within interstitial spaces  
between the interbonded grains of the hard material, at  
least a portion of the interbonded nanoparticles of  
non-carbide-forming material interbonded with the  
interbonded grains of hard material.

10. The polycrystalline compact of claim 9, wherein at least a portion of the interbonded nanoparticles of non-carbide-forming material further comprise at least one of molybdenum, osmium, ruthenium, rhodium, iridium, platinum, scandium tungstate, and zirconium tungstate.

11. A polycrystalline compact, comprising:  
a polycrystalline hard material comprising interbonded  
grains of diamond; and

## 16

interbonded nanoparticles comprising one or more  
elemental rhenium, elemental molybdenum, elemental  
osmium, elemental ruthenium, elemental rhodium,  
elemental iridium, elemental platinum, and an alloy  
thereof within interstitial spaces between the inter-  
bonded grains of diamond, at least a portion of the  
interbonded nanoparticles interbonded with the inter-  
bonded grains of diamond.

12. A method of forming a polycrystalline compact,  
comprising:

forming a polycrystalline hard material comprising inter-  
bonded grains of hard material; and  
forming interbonded nanoparticles of non-carbide-form-  
ing material within interstitial spaces between the inter-  
bonded grains of the hard material, at least a portion of  
the interbonded nanoparticles of non-carbide-forming  
material interbonded with the interbonded grains of  
hard material.

13. The method of claim 12, wherein forming a polycrys-  
talline hard material comprises:

forming nanoparticles of the non-carbide-forming mate-  
rial on particles of the hard material; and  
sintering the nanoparticles of the non-carbide-forming  
material and the particles of the hard material.

14. The method of claim 13, wherein forming nanopar-  
ticles of the non-carbide-forming material on particles of the  
hard material comprises functionalizing surfaces of at least  
one of the nanoparticles of the non-carbide-forming material  
and the particles of the hard material.

15. The method of claim 12, wherein forming a polycrys-  
talline hard material comprises:

forming an admixture comprising nanoparticles of the  
non-carbide-forming material and particles of the hard  
material; and  
sintering the admixture.

16. The method of claim 12, further comprising forming  
at least one of cobalt, nickel, and iron within at least a  
portion of the interstitial spaces.

17. The method of claim 16, wherein forming at least one  
of cobalt, nickel, and iron within at least a portion of the  
interstitial spaces comprises:

forming nanoparticles of the non-carbide-forming mate-  
rial on particles of the at least one of cobalt, nickel, and  
iron to form coated particles;  
combining the coated particles with particles of the hard  
material; and  
sintering the coated particles and particles of the hard  
material.

18. The method of claim 12, wherein forming interbonded  
nanoparticles of non-carbide-forming material comprises  
forming the interbonded nanoparticles of non-carbide-form-  
ing material to comprise one or more of elemental rhenium,  
elemental molybdenum, elemental osmium, elemental  
ruthenium, elemental rhodium, elemental iridium, elemental  
platinum, alloys thereof, scandium tungstate, and zirconium  
tungstate.

19. A method of forming a cutting element, comprising:  
forming a polycrystalline compact according to the  
method of claim 12; and  
attaching the polycrystalline compact to a substrate.

20. A method of forming an earth-boring tool, comprising:  
forming at least one cutting element according to the  
method of claim 19; and  
attaching the at least one cutting element to a body.